

# UNITED STATES PATENT OFFICE.

TAICHIRO YOSHIZAWA, OF TOKYO, JAPAN, ASSIGNOR TO NAIGWAI KAGAKU SEIHIN KABUSHIKI KWAIIHA, OF TOKYO, JAPAN.

## ANTICORROSION COMPOSITION.

1,365,760.

Specification of Letters Patent. Patented Jan. 18, 1921.

No Drawing.

Application filed August 26, 1919. Serial No. 320,012.

To all whom it may concern:

Be it known that I, TAICHIRO YOSHIZAWA, of Tokyo, Japan, subject of His Majesty the Mikado of Japan, have invented new and useful Improvements in Anticorrosive Compositions, of which the following is a specification.

This invention is an improved anti-corrosive composition for use in protecting metal and especially tools, instruments, machinery, pens and the like from rust.

One object of the invention is to provide an improved composition of this character, which is adapted to be used in an acid solution such as is employed for disinfecting metallic tools, instruments and the like, to prevent such tools or instruments from becoming oxidized or rusted and to also protect them from rust while in storage, transportation, or packed.

Another object of the invention is to provide an improved composition of this character which not only is an anti-corrosive, but which also prolongs the disinfecting power of a solution of mercuric chlorid, or the like.

Another object of the invention is to provide an improved composition of this character which is especially adapted to be mixed with an ink mainly made of tannic acid or sulfuric acid, to prevent the ink from corroding pens.

Another object of the invention is to provide an improved composition of this character which is adapted to prevent a steam boiler or other like boiler from scaling.

Another object of the invention is to provide an improved composition of this character which can be readily mixed and solved as needed, which can be produced at small cost, and which can be readily packed, transported, and stored.

My improved compound consists of comminuted borax and dextrin.

Dextrin, if dissolved in a moderate quantity of water, forms a solution of syrupy

viscosity and when borax is mixed therewith, forms a vehicle which carries the borax, holds the same in suspension and causes the borax to adhere to the applied metal surface. 50

I make a powder of borax and dextrin in the proportions of—

|         |               |
|---------|---------------|
| Borax   | 5 to 15 parts |
| Dextrin | 2 to 5 parts  |

55

To render ink such as is mainly made of tannic acid or sulfuric acid anti-corrosive, I mix with such ink about 1% of a powder of—

|         |               |
|---------|---------------|
| Borax   | 8 to 15 parts |
| Dextrin | 2 to 3 parts  |

60

The powder does not affect or change the color of the ink and is effective to render the ink anti-corrosive, so that it does not cause 65 pens used therewith to become foul and rusted.

To render mercuric chlorid solution in which tools and the like are immersed for disinfection and for cleansing purposes anti-corrosive, I mix therewith about 3% of a powder of—

|         |               |
|---------|---------------|
| Borax   | 5 to 10 parts |
| Dextrin | 2 to 5 parts  |

75

The powder not only renders the acid solution non-corrosive, but also greatly prolongs its disinfecting power.

My improved composition is also effective to prevent scaling in steam boilers, still 80 boilers, and the like.

Having thus described my invention, I claim:

1. The herein described anti-corrosive composition consisting of powdered borax 85 and dextrin.

2. The herein described anti-corrosive composition consisting of powdered borax 5 to 15 parts, and comminuted dextrin 2 to 5 parts.

TAICHIRO YOSHIZAWA.